

## UNITED STATES PATENT OFFICE

AUGUSTUS R. DE TARTAS, OF DOUGLAS MANOR, LONG ISLAND, NEW YORK

## PHOTOGRAPHIC REVERSAL PROCESS

No Drawing.

Application filed April 9, 1929. Serial No. 353,898.

This invention relates to a photographic process, known in the art as "reversal", in which positive pictures are made upon the same support and in the same emulsion that is exposed in the camera, which process comprises the development of the emulsion, after exposure in the camera, into a negative silver image, the removal of said silver image and the conversion of the remaining undeveloped silver salts in the emulsion into a positive image.

One disadvantage of prior processes has been that they have required extreme precision in the time of exposure in the camera.

Another disadvantage is that they have required accurate control of the formation of the final image at one or more of their stages. Improvements in the art directed to render a reversal process more practical in allowing greater latitude in the original exposure and involving a controlled production of the final image as a means to compensate for differences in the original exposure, have been counterbalanced to a certain extent by the

added disadvantage of rendering the process more expensive, longer and much more difficult to perform. These improved processes necessitate such additional steps as ascertaining the characteristics of the plate or film

before development of the emulsion into the final positive image or accurately timing the exposure to light of the sensitive silver salts remaining after the removal of the first negative image; but, in general, they require judgment and precision in the control of the production of the final image.

The present invention has for an object simplicity and time saving in the process, as it involves a minimum number of definite steps which remain at all times standard for a particular type of film. It also makes possible a reasonable latitude in the original exposure and the production of excellent positives of uniform quality, and the process may be carried out by an operator with no more than the usual care for the production of negatives, the extreme care in the control of the formation of the final positive image and the human judgment factor in arriving at the desired result being eliminated.

The present invention has for another object the total elimination of flashing of the emulsion or any exposure of the latter to white light at any stage in the process after initial exposure in the camera, the process being performed in the usual red light or in complete darkness, thus simplifying the process, reducing its cost and likewise relieving the operator of any undue care or responsibility in its performance. It may be remarked that the exposure of the emulsion to white light during the process of development has, in general, heretofore been a basic requirement of controlled "reversal" processes and has invariably involved the judgment of a skilled operator in the exposure or in the control of the formation of the final image, exception being had to processes utilizing special apparatus automatically performing such exposure or control of the formation of the final image.

According to the present invention positives of uniform quality may be produced by a series of standard steps performed in the usual red light or in total darkness. The following is an example of steps performed in the order of sequence stated embodying the present invention:—

1. Development of the emulsion, after exposure in the camera, into a negative silver image;
2. Placing the emulsion into a hypo fixing bath, which removes part of the undeveloped silver salts;
3. Reversal of the image, i. e. the bleaching or removal of the negative image;
4. Clearing the emulsion or removing the products formed in step 3 therefrom;
5. Redevelopment of the emulsion or conversion into a positive image;
6. Fixing the image in a hypo bath, or removing all undeveloped silver salts.

After each step of the process, as above stated, there will be the usual washing of the emulsion.

Another important improvement which my invention contemplates or makes possible is a standard timing factor for each of the steps, i. e. each step is performed in a definite period of time which remains the same

for a particular type of film. In this way the production of satisfactory results is automatically assured without extreme skill or care or judgment on the part of the operator.

5 Carrying out the removal of part of the undeveloped salts, prior to the reversal of the image is deemed to be one of the important features of the present invention. Heretofore, in processes which involved this step 10 of partial removal of undeveloped salts, the latter has been performed after the developed silver image has been bleached or removed and in certain cases in the open light and has involved considerable skill and judgment in 15 its control and in the control of other steps associated with these processes in the formation of the final image.

15 The partial fixing of the first negative image in the emulsion or partial removal of undeveloped salts, performed after the development of the emulsion into a silver image and before the removal of the latter, enables the process to be carried on without exposure to white light of any kind and with no other 20 control than the allotment of definite standard times to the several steps of the process.

25 While the process is applicable to any type of emulsion including "negative" emulsions, it produces particularly satisfactory results 30 when using a "positive" emulsion.

An example of the process will now be described as applied to a motion picture film consisting of a support of a cellulose composition with a "positive" emulsion thereon.

35 *Step 1.*—The film is first exposed in the usual manner in a camera. Although it is evidently desirable that this exposure be carefully timed, no more than the usual care 40 exercised in the exposure to light of films for the production of negatives is necessary. The emulsion is then caused to be developed to a negative image which may be done by any of the well known developers. However 45 it is preferred to use a solution of the following composition:

*Developer stock solution*

|                                       |            |
|---------------------------------------|------------|
| Water                                 | 64 ounces  |
| 50 Monomethyl paramidophenol sulphate | 120 grains |
| Sodium sulphite                       | 3½ ounces  |
| Hydrochinon                           | 480 grains |
| Sodium carbonate                      | 5½ ounces  |

55 It is noted that the usual restrainer such as potassium bromide is omitted. This developer without restrainer is quick in its action upon the exposed silver salts within the emulsion 60 and permits said exposed silver salts to blacken freely and to a full degree.

One ounce of the stock solution is added to three ounces of water for use in developing the silver image and the time factor or 65 period of immersion of the film in this bath

is five minutes. The film is then rinsed for a short time.

*Step 2.*—The film is placed in a fixing bath which is made as follows:

*Fixing stock solution*

|                              |           |
|------------------------------|-----------|
| Water                        | 32 ounces |
| Sodium thiosulphate ("hypo") | 1 ounce   |
| Sodium sulphite              | ½ ounce   |
| Formalin                     | 10 minims |

75 75

Or, as an alternative, any well known acid fixing solution is made up and set aside as a stock solution.

The film is placed into a bath consisting of 6 ounces of the stock solution and 32 80 ounces of water, the period of immersion being five minutes, and is then given a thorough washing such as in running water for about five minutes.

*Step 3.*—The film is then submitted to a bleaching or reversing bath whereby the blackened image is removed. This bath consists of 32 ounces of water and two ounces of the following solution:

*Reversing stock solution*

|                               |                   |
|-------------------------------|-------------------|
| Water                         | 8 ounces          |
| Potassium bichromate          | 194 grains        |
| Sulphuric acid (concentrated) | 6 drams 30 minims |

95 95

The film is left in the reversing bath for two minutes and is then washed with water. Other known bleaching or reversing agents may be used but it has been found that none 100 of the latter give results as satisfactory as the one outlined above.

*Step 4.*—The film is placed in a clearing bath which removes the products formed in step 3 and which consists of

|                    |           |
|--------------------|-----------|
| Water              | 32 ounces |
| Sodium bisulphite  | 1 ounce   |
| Sodium bicarbonate | 1 ounce   |

105 105

It has also been determined that this acid 110 clearing bath is better adapted for clearing purposes than an alkali bath and to produce excellent results. The time factor in this step is three minutes when using the particular clearing bath described, the film being then again washed with water.

*Step 5.*—The remaining salts in the emulsion are now caused to be redeveloped or converted into a positive image. While the solution used in step 1 is very desirable for 115 this redevelopment step, any known developer or blackening reagent that will bring out the positive image in a satisfactory manner may be used. The period of immersion of the film, for this step, in the solution of step 1, is five minutes, which is followed by a rinsing of the film.

*Step 6.*—The film is placed in a regular hypo fixing bath to remove all undeveloped silver salts or other unused products or im-

120 125 130

purities. The time factor for immersion of the film in this step is ten minutes, the film having the final positive image thereon being then thoroughly washed and dried in the usual manner.

In each of the steps described the film is kept in motion in the solutions or the latter are caused to be agitated. It is of course understood that, if so desired, the strength of the solutions may be varied, the timing factors in each step being correspondingly varied to produce the same desired results. However, it is essential to carry out the process in the exact sequence or order of the steps given herein. The solutions described in connection with my process remain in good working order and may be reused for succeeding films until exhausted.

In practice, the strengths of the various solutions and the periods of immersion of the emulsion therein are first determined by test for a particular type or make of emulsion. The process makes it then possible to develop emulsions similar to that of the test, but which may have been exposed to light under various circumstances, with the same certainty of satisfactory results, the strengths of the various solutions and the timing factors for each step remaining always the same. In this way, the process may be automatically carried out with great simplicity and with no more than the usual care in developing negatives.

This simplicity in the process is evidently made possible by the particular sequence of steps, performed without exposure to light, which also makes possible a reasonable latitude in the original exposure in the camera.

The described process is an improvement of substantial value in its simplicity, low cost and total elimination of extreme care or skill on the part of the operator. The number of steps is a minimum, since the process eliminates re-exposure of the emulsion to a controlled light or to a white light of any kind or ascertaining the printing characteristics of the emulsion. It makes possible the production of positives of excellent and uniform quality, without requiring either extreme precision in the original exposure or extreme skill in the development of the emulsion. After having once determined the strengths of the solutions in the various steps and the timing factors of each step for a particular type of film, succeeding films of the same type, regardless of the circumstances under which they are exposed, are developed with the same strengths of solutions and timing factors and with the same accuracy in the final result.

While the development of a motion picture film has been chosen for convenience in describing the invention, it is understood that the latter is of a general character and is applicable in like manner to films, plates,

prints and the like. In this respect, steps 5 and 6 may be changed to comprise or include any of the toning baths or any of the many processes known to photographers as a means to impart the final image to the emulsion.

I claim:

1. In a photographic process of making positive images in the same emulsion as originally exposed in the camera, the following steps to be performed in their order of sequence: (1) developing the emulsion after exposure in the camera into a negative image, (2) removing part of the undeveloped salts remaining in the emulsion and (3) removing the negative image from the emulsion.

2. In a photographic process of making positive images in the same emulsion as originally exposed in the camera, the following steps, performed without exposure to white light and in their order of sequence: (1) developing the emulsion after exposure in the camera into a negative image (2) removing part of the undeveloped salts remaining in the emulsion and (3) removing the negative image from the emulsion.

3. In a photographic process of making positive images in the same emulsion as originally exposed in the camera, in which process the emulsion is developed into a negative image and said image is removed, the step of removing part of the undeveloped salts, remaining in the emulsion after its development into a negative image, performed before the removal of the negative image.

4. In a process of making positive images in the same emulsion as originally exposed in the camera, in which process the element is developed into a negative image and said image is removed, the step of removing part of the undeveloped salts from said element after the development of the negative image and before the removal of the silver image, said step being performed without exposure to white light and in a definite period of time which remains constant for a particular type of film.

5. In a process of making photographic positive images by reversal from photographic negative images in a light sensitive element, in which process the element is developed into a negative image and said image is removed, the step of partially fixing said negative image performed before its removal and in a period of time which remains constant for a particular type of emulsion.

6. A process of making photographic positive images by reversal from photographic negative images comprising the following steps, performed in their order of sequence: (1) developing the exposed emulsion into a negative image (2) partially removing undeveloped salts from the emulsion (3) removing the negative image from the emulsion and (4) redeveloping the remaining emulsion into the final positive image.

7. A process of making photographic positive images by reversal from photographic negative images comprising the following steps, performed without exposure to white light and in their order of sequence: (1) developing the exposed emulsion into a negative image (2) placing the emulsion in a fixing bath to partially remove undeveloped salts from the silver image (3) removing the silver image from the emulsion and (4) redeveloping the remaining emulsion into the final positive image.

8. A process of making photographic positive images by reversal from photographic negative images comprising the following steps, performed without exposure to white light and in their order of sequence: (1) developing the exposed emulsion into a negative image (2) partially removing undeveloped salts from the emulsion (3) removing the negative image from the emulsion (4) clearing the latter from the products formed during the removal of the negative image and (5) redeveloping the remaining emulsion into the final positive image.

9. A process of making photographic positive images by reversal from photographic negative images comprising the following steps, performed without exposure to white light and in their order of sequence: (1) developing the exposed emulsion into a negative image (2) partially removing undeveloped salts from the emulsion (3) removing the negative image from the emulsion (4) clearing the latter from the products formed during the removal of the negative image (5) developing a positive image in the emulsion and (6) removing from the latter all undeveloped salts.

10. A process of making a photographic image by reversal from a photographic negative image in a "positive" emulsion which comprises partially removing undeveloped salts from the emulsion after the latter is developed into a negative image, removing the latter, and redeveloping the remaining emulsion into the positive image, each of said steps being performed without exposure to white light and in a definite period of time.

11. A process of making a photographic image by reversal from a photographic negative image in a sensitive element which comprises, as sole steps in the process: (1) developing the emulsion into a negative image (2) partially fixing said image (3) removing said image (4) removing the products formed while removing said image and (5) redeveloping the remaining emulsion into a positive image; all of said steps being performed without exposure to white light and each in a definite period of time which remains constant for a particular type of film.

In testimony whereof, I have affixed my signature to this specification.

AUGUSTUS R. DE TARTAS.